

# United States Patent Office

2,695,270

Patented Nov. 23, 1954

1  
2,695,270

## OIL SOLUBLE CATIONIC TEXTILE ANTISTATIC AGENT

George D. Jefferson, Kennett Square, Pa., and Allen V. Riley, Jr., New Castle, Del., assignors to Atlas Powder Company, Wilmington, Del., a corporation of Delaware

No Drawing. Application March 22, 1951,  
Serial No. 217,067

17 Claims. (Cl. 252—8.7)

The present invention relates to a novel composition of matter. More specifically it relates to a novel textile treating composition.

It is an object of the present invention to provide an oil base, anti-static finish for textiles.

It is another object of the present invention to provide a textile treating composition for containing an oil solubilized cationic surface active agent.

It is a further object of the present invention to provide textiles which are rendered anti-static by application thereto of an oil containing a cationic surface active agent solubilized therein.

These and other objects will become apparent in the course of the following specification and claims.

Adaptability of fibers, staple fibers, felts, cords, threads, yarns, pellicles, filaments, fabrics and the like to automatic handling operations is of extreme importance in the manufacture of textiles. Modern high speed machinery technique requires a feed of appropriate characteristics to permit uninterrupted and fault free operation. The electrostatic qualities of the textile being handled can frequently spell the success or failure of such undertakings. Thus, yarn which tends to "balloon," due to the accumulation of static charges as it passes over equipment, is entirely unsatisfactory for operations such as knitting where it produces uneven stitches and knotting. Furthermore, in the spinning of yarns, the presence of static electrical charges upon the particles being spun, will cause production of uneven yarns and a high percentage of slubs. The lubricity of the textile being processed is another factor of prime importance in textile machine operations. Whether in the form of fibers, staple fibers, felts, cords, threads, yarns, pellicles, continuous filaments, fabrics or other, it is necessary that the internal and external abrasive and frictional tendencies of the particles toward one another and toward the surfaces over which they pass, be reduced to the minimum. It has, therefore, become the practice of the trade to apply oils to textiles at various stages during processing to obtain the desired lubricity.

In accordance with the present invention it has been discovered that a very useful textile finish which supplies both lubricity and anti-staticity can be prepared by solubilizing in oil a member of a class of organic morpholine derivatives as described below:

The morpholine derivatives which act as textile anti-static agents are materials of the class



wherein R is a long-chain aliphatic radical containing from 11 to 20 carbon atoms and A is an anion. Suitable derivatives may be formed by substituting within the above formula, the components suggested in Table I.

TABLE I

| R        | Lower Alkyl | A            |
|----------|-------------|--------------|
| Undecyl  | Methyl      | Halide       |
| Lauryl   | Ethyl       | Nitrate      |
| Myristyl | Amyl        | Phosphate    |
| Cetyl    |             | Alkylsulfate |
| Oleyl    |             | Cyanide      |
| Stearyl  |             | Acetate      |
| Soyalyl  |             | Benzoate     |
|          |             | Citrate      |
|          |             | Tartrate     |

2

By the "soyaly" radical is meant the mixture of aliphatic hydrocarbon radicals obtainable by changing —COOH to —CH<sub>2</sub>— in the mixture of fatty acids occurring as glycerides in soyabean oil. It is obvious that derivatives of other mixed fatty acids obtained from naturally occurring oils of animal and vegetable origin are likewise suitable as are mixed fatty and rosin acid derivatives as obtained from tall oil. These materials are fully disclosed in the prior art and their preparation need not be elaborated here.

Since the organic morpholine derivatives described above are essentially oil immiscible, it is necessary to dissolve them in "solubilizing agent" prior to their addition to the oil. It has been found that polyoxyethylene derivatives of long chain organic compounds containing active hydrogen are useful for this purpose. The materials which have been found particularly valuable in this capacity are the \*4 to 20 polyoxyethylene derivatives of long chain acids, alcohols, amides and amines which contain from 11 to 20 carbon atoms and the 4 to 20 polyoxyethylene derivatives of partial esters of the above described long chain acids with polyols. These compounds may be expressed by the structure



wherein RY represents undecyl, lauryl, myristyl, cetyl, oleyl, stearyl radicals, the natural mixed fatty and/or rosin acid radical derivatives such as soyaly, tall oil and the like as described above; x is a number from 4 to 20 inclusive, Y representing the terminal carbon, substituted as expressed in Table II.

TABLE II

| 35 | Y | Structural formula: RY(C <sub>2</sub> H <sub>4</sub> O) <sub>x</sub> H |
|----|---|------------------------------------------------------------------------|
| 40 |   |                                                                        |
| 45 |   |                                                                        |
| 50 |   |                                                                        |
| 55 |   |                                                                        |
| 60 |   |                                                                        |
| 65 |   |                                                                        |
| 70 |   |                                                                        |

In Table II above A is the residue of a polydric alcohol containing at least three carbon atoms or a cyclic inner ether thereof and R' is an aliphatic organic radical.

Compounds containing the partial ester linkage include polyoxyethylene sorbitan mono-, di-, and tri-laurate, palmitate, stearate and oleate. A particularly valuable solubilizing agent may be formed by employing a partial ester of a higher fatty acid with a hexitol or hexitol inner ether in combination with the polyoxyethylene derivatives discussed above. Substances such as partial esters of sorbitol and sorbitan, mannitol and mannan and the like may be used in such mixtures.

The oils employed as the base of the composition may

\* Figure refers to average number of mols of polyoxyethylene groups per mol of acid, alcohol, amide, or amine.

## 3

be of the conventional petroleum base, lubricating grade. Their viscosities may vary through wide ranges depending upon the anticipated application. A particularly suitable oil for textile treatment is refined mineral oil having a viscosity of 50 Saybolt Universal seconds at 100° F. Such oils are available commercially from major oil companies and textile supply houses and are sold under such trade-marks as Sunvis 11, Topaz A and Absorbent K. Other oils of animal and vegetable origin may also be used for specialized applications.

The components are combined by melting the organic morpholinium compound and the solubilizer together. After solution is obtained, the oil is added with agitation. Frequently, it is advisable to warm the mineral oil slightly (to about 60° C.) prior to its addition. A few drops of water may be added to obtain a clear solution if the composition appears cloudy.

The proportion of components may vary widely depending on the nature of the textile and the particular operation for which it is being prepared. In general, the oil component may comprise from 70 to 90% of the final composition. The organic morpholinium derivative has been found effective at concentrations as low as 3%. However, 10% or more may be solubilized and suitably applied. The solubilizing component composes 7 to 20% of the finished composition and must be at least equal by weight to the amount of organic morpholinium derivative employed. Where a combination of polyoxyethylene derivatives and partial esters of long chain fatty acids with polyols is employed, the ratio of these components may vary from 35:65 to 65:35.

The following examples are listed to illustrate the invention. They are not intended to limit it in any way.

## Example I

A nylon coning oil containing 10% of 4 polyoxyethylene stearic acid, 4% of cetyl ethyl morpholinium ethosulfate and 86% of 50 Saybolt refined mineral oil is prepared by melting the organic morpholinium anti-static agent and solubilizer together at 60° C. The mineral oil is heated to the same temperature and added with constant agitation.

Following the procedure of Example I the following compositions may be prepared:

## COMPOSITION

| Example | Mineral Oil Percent | Anti-static agent                              | Solubilizer                                                                                     |
|---------|---------------------|------------------------------------------------|-------------------------------------------------------------------------------------------------|
| II      | 86                  | 4% of cetyl ethyl morpholinium ethosulfate.    | 10% of 5 polyoxyethylene octadecylamine.                                                        |
| III     | 86                  | do                                             | 10% of 5 polyoxyethylene lauryl alcohol.                                                        |
| IV      | 86                  | do                                             | 3.5% of 20 polyoxyethylene sorbitan monolaurate and 6.5% of sorbitan monoleate.                 |
| V       | 86                  | do                                             | 3.5% of 20 polyoxyethylene sorbitan monoleate and 6.5% of sorbitan monoleate.                   |
| VI      | 78.7                | 3.1% of cetyl ethyl morpholinium ethosulfate.  | 9.5% of 10 polyoxyethylene sorbitan monolaurate and 7.6% of sorbitan monolaurate in 1.1% water. |
| VII     | 86.6                | 3.4% of cetyl ethyl morpholinium ethosulfate.  | 5% of 10 polyoxyethylene tall oil acids and 5% of sorbitan monoleate.                           |
| VIII    | 85.0                | 5% of cetyl ethyl morpholinium ethosulfate.    | Do.                                                                                             |
| IX      | 84.0                | 6% of cetyl ethyl morpholinium ethosulfate.    | Do.                                                                                             |
| X       | 83.0                | 7% of cetyl ethyl morpholinium ethosulfate.    | Do.                                                                                             |
| XI      | 82.0                | 8% of cetyl ethyl morpholinium ethosulfate.    | Do.                                                                                             |
| XII     | 80.0                | 10% of cetyl ethyl morpholinium ethosulfate.   | Do.                                                                                             |
| XIII    | 70.0                | 10% of soyalyl ethyl morpholinium ethosulfate. | 20% of 8 polyoxyethylene lauryl amide.                                                          |
| XIV     | 90.0                | 3% of lauryl methyl morpholinium methosulfate. | 7% of 4 polyoxyethylene oleic acid.                                                             |

These lubricating anti-static compositions may be ap-

plied to the textile by the same means and with the same equipment conventionally employed for oil application. To minimize electrostatic tendencies to a workable extent, it has been found desirable in extreme cases of which nylon is an example to deposit enough finish to comprise about 2% to 3% by weight of finish based on final treated textile. Where the static problem is not so acute, such as in the case of viscose rayon, as little as 1% is effective. After the finishing composition has been applied and air dried it may be evaluated for electrostatic properties by rubbing twelve times with a glass rod to induce a charge and then, after observation and grounding, rubbing twelve times with a hard rubber rod to induce an opposite charge. Observations are given electrostatic ratings as indicated in Table II.

Table II

| Rating | Observation                                                                  |  |  |
|--------|------------------------------------------------------------------------------|--|--|
| 0      | No evidence of electrostatic charge.                                         |  |  |
| 1      | Just enough electrostatic charge to disturb a filament.                      |  |  |
| 2      | Sufficient electrostatic charge to lift a filament from a skein.             |  |  |
| 3      | Sufficient electrostatic charge to cause a slight ballooning of a skein.     |  |  |
| 4      | Sufficient electrostatic charge to cause considerable ballooning of a skein. |  |  |

In the following tests, the compositions are applied to 30 denier 7 filament nylon using a single end nylon sizing machine at the various applicator roll speeds as indicated.

| Example | Composition | Applicator Roll speed (R. P. M.)                                                                                             | Electrostatic Rating |     |
|---------|-------------|------------------------------------------------------------------------------------------------------------------------------|----------------------|-----|
|         |             |                                                                                                                              | -                    | +   |
| 35      |             |                                                                                                                              |                      |     |
| 40      | XV          | 36.6% of refined mineral oil.<br>3.4% of cetyl ethyl morpholinium ethosulfate.<br>5.0% of 10 polyoxyethylene tall oil acids. | 6                    | 2 1 |
|         | XVI         | 5.0% of sorbitan monoleate.<br>Same as Example XV.                                                                           | 6                    | 1 0 |
|         | XVII        | Same as Example XV.                                                                                                          | 9                    | 0 0 |
| 45      | XVIII       | 82.0% of refined mineral oil.<br>8.0% of cetyl ethyl morpholinium ethosulfate.<br>5.0% of 10 polyoxyethylene acid.           | 3                    | 0 0 |
|         | XIX         | 5.0% of sorbitan monoleate.<br>Same as Example XVIII.                                                                        | 6                    | 0 0 |
| 50      | XX          | Same as Example XVIII.                                                                                                       | 9                    | 0 0 |

While nylon has been demonstrated in detail above, other textiles may be finished in a similar manner. Electrostatic properties of several are demonstrated below:

| Example | Textile                                                      | Electrostatic Ratings                    |           |   |     |
|---------|--------------------------------------------------------------|------------------------------------------|-----------|---|-----|
|         |                                                              | Treated <sup>1</sup>                     | Untreated | - | +   |
| 60      |                                                              |                                          |           |   |     |
| XXI     | Acrylic fibre "Chemstrand" (A single ends yarn of 48 count). | 0                                        | 0         | 3 | 4   |
| 65      | XXII                                                         | Viscose rayon (150 denier, 40 filament). | 0         | 0 | 3 3 |
|         | XXIII                                                        | Acetate rayon (150 denier, 40 filament). | 0         | 0 | 4 4 |
|         | XXIV                                                         | Spun glass fibre.                        | 0         | 0 | 4 4 |

70 <sup>1</sup> By single end application of the composition described in Example XII followed by air drying.

The compositions are widely useful for the purpose described above for textiles of synthetic or natural origin. It may be applied to fibers, staple fibers, felts, cords, threads, yarns, pellicles, filaments, fabrics and the like to textiles of animal, vegetable, mineral and synthetic origin. Among such substances may be mentioned cellulose acetate, regenerated cellulose, acrylic polymers and copolymers, vinyl polymers and copolymers, mixed copolymerization products of dibasic acids such as those of adipic acid and hexamethyldiamine, vinylidene, chloride polymers, the synthetic proteins, cotton, wool, glass, linen, asbestos and the like. The composition is also useful in the treating of hair.

85 It will be apparent to those skilled in the art that many

variations are possible without departing from the scope of the invention.

We claim:

1. An oil soluble composition of matter comprising a compound of the formula:



wherein R is a long chain aliphatic hydrocarbon radical containing from 11 to 20 carbon atoms and A is an anion, and as an oil solubilizer therefor a polyoxyethylene derivative with from 4 to 20 oxyethylene groups of a long chain organic compound containing from 11 to 20 carbon atoms and an active hydrogen, said organic compound being selected from the group consisting of alcohols, acids, amides and amines, present in the proportion of 3 to 10 parts by weight of the first ingredient and 7 to 20 parts by weight of the second ingredient.

2. The composition of matter as defined in claim 1 wherein the long chain organic compound containing active hydrogen is an alcohol.

3. The composition of matter as defined in claim 1 wherein the long chain organic compound containing active hydrogen is an acid.

4. The composition of matter as defined in claim 1 wherein the long chain organic compound containing active hydrogen is an amide.

5. The composition of matter as defined in claim 1 wherein the long chain organic compound containing active hydrogen is an amine.

6. A composition of matter as defined in claim 1 wherein A is an ethosulfate radical.

7. An oil soluble composition of matter comprising from 3 to 10 parts of a compound of the formula:



wherein R is a long chain aliphatic hydrocarbon radical containing from 11 to 20 carbon atoms and A is an anion, and as an oil solubilizer therefrom from 7 to 20 parts of a mixture of a polyoxyethylene derivative with from 4 to 20 oxyethylene groups of a long chain organic compound containing from 11 to 20 carbon atoms and an active hydrogen, said organic compound being selected from the group consisting of alcohols, acids, amides and amines, and a hexitan partial ester of a long chain fatty acid, the ratio of the components of said mixture being from 35:65 to 65:35.

8. A textile bearing a composition containing from 70% to 90% of a mineral oil, from 3% to 10% of a compound of the formula:



- wherein R is a long chain aliphatic hydrocarbon radical containing from 11 to 20 carbon atoms and A is an anion, and from 7% to 20% of a member of the class consisting of a polyoxyethylene derivative with from 4 to 20 oxyethylene groups of a long chain organic compound containing 11 to 20 carbon atoms and an active hydrogen, said organic compound being selected from the group consisting of alcohols, acids, amides and amines, and a mixture of said polyoxyethylene derivative in conjunction with a hexitan partial ester of a long chain fatty acid, the ratio of the components of said mixture being from 35:65 to 65:35.
9. The textile as defined in claim 8 wherein the textile is nylon.
10. The textile as defined in claim 8 wherein the textile is rayon.
11. The textile as defined in claim 8 wherein the textile is an acrylic polymer.
12. The textile as defined in claim 8 wherein the textile is glass.
13. The textile as defined in claim 8 wherein the textile is a synthetic protein.
14. The textile as defined in claim 8 wherein the long chain organic compound containing active hydrogen is an alcohol.
15. The textile as defined in claim 8 wherein the long chain organic compound containing active hydrogen is an acid.
16. The textile as defined in claim 8 wherein the long chain organic compound containing active hydrogen is an amide.
17. The textile as defined in claim 8 wherein the long chain organic compound containing active hydrogen is an amine.

35

#### References Cited in the file of this patent

#### UNITED STATES PATENTS

| Number    | Name             | Date           |
|-----------|------------------|----------------|
| 1,970,578 | Schoeller et al. | Aug. 21, 1934  |
| 2,186,628 | Dickey           | Jan. 9, 1940   |
| 2,191,922 | Bruson           | Feb. 27, 1940  |
| 2,261,002 | Ritter           | Oct. 28, 1941  |
| 2,297,221 | Huttenlocher     | Sept. 29, 1942 |
| 2,404,240 | MacLaurin        | July 16, 1946  |
| 2,417,992 | Niederl et al.   | Mar. 25, 1947  |
| 2,492,394 | Olpin et al.     | Dec. 27, 1949  |
| 2,565,503 | Sproule et al.   | Aug. 21, 1951  |

#### OTHER REFERENCES

- 50 Atlass, "Spans and Tweens," 1942, pp. 1-3. (Copy in Div. 64.)  
 Atlass, Surface Active Agents, 1948. (Copy in Div. 64.)

55

60